

## UNITED STATES PATENT OFFICE

2,245,747

METHOD OF TREATING CENTRIFUGAL  
METAL MOLDS

Clarence Dale Barr, Birmingham, Ala., assignor to  
American Cast Iron Pipe Company, Birmingham, Ala., a corporation of Georgia

No Drawing. Application July 24, 1939,  
Serial No. 286,284

6 Claims. (Cl. 22—189)

This invention relates to a method of treating centrifugal metal molds, as of steel or cast iron, for use in the centrifugal casting of iron or steel pipes, tubes, and the like.

In the centrifugal casting of iron or steel pipes, tubes, etc., it is customary to provide the mold with a relatively thin coating to protect the mold against injury from the molten metal and thereby prolong its life, and also to minimize chilling at the surface of the casting, to facilitate separation of the casting from the mold, etc. A common procedure is to treat the surface of the mold with a powder in a finely divided condition which may be introduced into the mold by a screw conveyor, a tilting trough or an air-blast nozzle, centrifugal force being usually relied upon in whole or in part to effect the desired distribution of the coating material over the surface of the mold. This coating material is commonly applied to the mold surface just ahead of the stream of molten metal. It has also been proposed to introduce coating materials in the form of pastes or liquids sprayed or blown onto the surface of the rotating mold, usually just ahead of the molten metal, with reliance on centrifugal force in whole or in part to effect the distribution of the coating material. A wide variety of coating materials have also been proposed, including finely divided graphite or lamp black either mixed with a carrier or applied directly to the surface of a coating of refractory material separately applied.

Difficulties have been experienced, with the procedures heretofore employed, in securing a uniform distribution of the coating material. Powder and paste, though blown into the mold, are not distributed equally over the surface of the mold, even though the distribution is aided by centrifugal force, with the result that variations in the thickness of the coating occur, producing spots on the mold surface which are not adequately protected and sometimes bare. This not only results in irregularities at the mold surface, but also the variations in coating thickness produce variations in the chemical and physical characteristics of the surface of the casting because of the consequent variations in the heat insulating characteristics of the coating, variations in the absorption of carbon, etc. Such variations furthermore militate against the production of a smooth, bright surface at the face of the casting, and if the mold is one for producing a design or special configuration at the surface of the casting, the details of the mold surface are not accurately reproduced in the casting because of variations of thickness at the irregu-

larities in the surface of the mold. Even though a liquid be employed for distributing the coating material on the face of the mold as heretofore proposed, there is a tendency for the particles suspended in the liquid to have an irregular distribution therein because of the action of gravity thereon or the tendency to agglomerate, so that even a fairly uniform distribution of the vehicle over the face of the mold does not produce a uniform distribution of the solid material after the vehicle has been vaporized. Difficulties have also been experienced in the clogging of the nozzles used with the coating materials heretofore employed.

15 I have discovered that the difficulties heretofore encountered in the use of the coating materials heretofore proposed as applied in the several suggested ways for coating the surface of metal molds used in the centrifugal casting of iron and steel pipes, tubes and the like, may be overcome, and materially improved results obtained, by proceeding in accordance with the method herein-after described.

It is therefore an object of this invention to 25 provide an improved method for treating the surfaces of metal molds used in the centrifugal casting of iron or steel pipes, tubes and the like, which will enable the coating material to be distributed over the entire surface of the mold with substantial uniformity.

Another object of this invention is to provide a 30 method of the type characterized which will produce a coating that lengthens the life of the mold.

Another object of this invention is to provide a 35 method of the type characterized which will produce a coating having substantially the same heat insulating characteristics throughout the surface of the mold.

Another object of this invention is to provide a 40 method of the type characterized which will produce a coating of the mold that is firmly adhesive to the mold surface, and which will not crack, flake, blister, or be roughened or displaced by contact of the molten metal therewith.

Another object of this invention is to provide a 45 method of the type characterized wherein the coating is stable and inert and protects the surface of the mold from oxidation or corrosion.

Another object of this invention is to provide a 50 method of the type characterized wherein the coating does not tend to cause the casting to stick thereto, but which acts as a lubricant to facilitate separation of the casting from the mold.

Another object of this invention is to provide a 55 method of the type characterized which employs

a coating material that does not tend to separate into its constituent materials and thereby produce an irregular distribution of the solid material in the liquid vehicle employed.

Another object of this invention is to provide a method of the type characterized which utilizes a coating material that can be sprayed without danger of clogging the nozzle and which flows or spreads easily on the surface of the mold so as to produce a substantially uniform distribution of the coating material thereover.

Another object of this invention is to provide a method of the type characterized whereby the mold is provided with a smooth glazed surface and the casting accordingly has a smooth surface, with a polished appearance, which is relatively free from blemishes and therefore of materially improved appearance over that heretofore obtained from casting in centrifugal molds.

Another object of this invention is to provide a method of the type characterized wherein the coating is highly resistant to brushing, scraping or other mechanical action.

Another object of this invention is to provide a method of the type characterized wherein the coating does not tend to build up materially on the mold surface and therefore avoids "caking" of the mold surface.

Another object of this invention is to provide a method of the type characterized which enables the accurate reproduction of fine detail in the mold design, even in the production of relatively intricate castings.

Another object of this invention is to provide a method of the type characterized which avoids the formation of gases from the coating material that tend to produce blow holes or gas pockets in the casting during the pouring of the molten metal.

Another object of this invention is to provide a method of the type characterized wherein the coating is relatively inert chemically and therefore does not react to any great extent with the molten metal.

Another object of this invention is to provide a method of the type characterized wherein the coating serves to reduce the chilling of the casting by reason of its heat insulating characteristics, and wherein this insulating effect is substantially uniform throughout the surface of the casting.

Another object of this invention is to provide a method of the type characterized which may be effectively applied either to a hot or a cold mold, and which also employs a coating material which can be applied by brushing or spraying, and which can also be applied under the most efficacious and most efficient conditions to obtain desired results.

Another object of this invention is to provide a method of the type characterized which by successive treatments of the mold surface produces a coating thereon which materially increases the life of the mold and improves the surface character of the casting.

Another object of this invention is to provide a method of the type characterized which is productive of a casting having a materially improved appearance.

Other objects will appear as the description of the invention proceeds.

I have discovered that a metal mold for the centrifugal casting of iron or steel pipes, tubes, etc., may be provided with a superior coating, productive of a superior casting, and carrying

into effect the foregoing objects, by applying to the surface thereof a coating of colloidal graphite in dilute solution or suspension in a volatile liquid. Any suitable liquid vehicle for said colloidal graphite may be employed, but at the present I prefer to use a mineral oil. Before application said mixture is preferably diluted by any suitable liquid miscible therewith, kerosene being at the present preferred, so as to produce a relatively dilute mixture or solution. But while an oil vehicle is preferred, the invention is not limited thereto.

The mold may be coated with the colloidal-graphite and mineral-oil mixture in any suitable way, as for example by brushing, but I prefer to apply the same by means of a spray nozzle, and while the coating of this invention may be applied while the mold is cold I prefer to apply the coating while the mold is hot, for example at 400° F. or above, so as to increase the rate of volatilization of the vehicle and therefore decrease the time consumed before the mold is ready for use. When the mold is coated while hot the liquid vehicle should preferably be one of low specific heat so as not to over-chill the mold, and therefore the mineral-oil-colloidal-graphite mixture diluted with kerosene hereinbefore mentioned has been found particularly satisfactory.

The coating of the present invention is preferably applied immediately after a casting operation so as to take advantage of the heat then present in the mold. Contrary to prior practice, the coating material is not applied immediately ahead of the introduction of the molten metal into the mold, but to insure that the volatile vehicle shall have become entirely volatilized in advance of the introduction of the molten metal and thereby eliminate the danger of gas pockets or blow holes due to volatilization of residual vehicle upon contact of the molten metal therewith, the coating is preferably applied immediately after a previous use to the mold and while it is still hot.

The colloidal-graphite-mineral-oil mixture may be applied in any suitable way, as by a spray nozzle delivering the liquid throughout three hundred and sixty degrees of arc while relative movement is effected axially of the mold between the mold and the spray nozzle, or a nozzle producing a lesser arc of spray may be used if relative rotation is maintained between the mold and the spray while relative axial movement is maintained therebetween, so that the spray travels in the form of a helix over the entire surface of the mold. In the latter event the spray preferably has a substantial spread in the direction of the axis of the mold, and the rate of rotation between the spray and mold, whether the spray is rotated or the mold is rotated, and the rate of axial movement between the spray and mold, whether the spray is advanced within the mold or the mold is advanced over the spray, are so correlated that the jet of sprayed material is progressively advanced in a spiral or helical path over the entire surface of the mold and at a uniform speed so that all portions of the mold receive equal quantities of the colloidal suspension. As the particles of graphite in such colloidal suspension are uniformly distributed through the liquid vehicle, the distribution of the graphite is accordingly uniform over the surface of the mold, and not irregular as in the case of liquid mixtures employ-

ing larger particles which may tend to separate from or agglomerate within the vehicle.

Any suitable pressure may be used for ejecting the colloidal suspension, suitable pressures having been found to be between forty and sixty pounds per square inch of air pressure. But although particular values as to temperature, pressure, etc., have been suggested it is to be expressly understood that the invention is not restricted thereto, as the temperature of the mold may be varied with regard to the speed with which the coating material is supplied, the pressure on the spray may be varied with the type of nozzle used and also with respect to the speed of relative movement between the spray and the surface of the mold, etc., so as to predetermine the quantity of coating material deposited on each square inch of mold surface, and the rate of relative rotation between the spray and mold and the rate of axial movement between the spray and mold may be correlated with the size of the jet and rate of passage through the nozzle, all so as to obtain the desired coverage of the mold surface and thickness of coating desired.

Owing to the fluidity of the coating material and the uniform distribution of the colloidal graphite therethrough, the resulting coating of graphite on the mold surface, after volatilization of the vehicle, is uniform over the surface of the mold. It is to be noted that centrifugal force is not relied upon to obtain the distribution of the coating material, but the coating material, which itself has uniform characteristics, is so applied as to produce a uniform deposit of the graphite in colloidally-small particles all over the surface of the mold. Owing to the fineness of the particle size of the deposited graphite it is capable of and does fill up the surface irregularities unavoidably present in the surface of a metal mold, and thereby the mold is provided with a smooth glazed surface which in turn results in the production of a casting whose surface is smooth and shiny, and therefore of materially superior appearance to that heretofore obtained. The graphite functions as a lubricant in facilitating separation of the casting from the mold, whereby sticking is avoided, and as the method of the present invention assures a uniform distribution of the coating material there is no burning through of the molten metal, or sticking of the casting to the mold, such as is likely to arise if thin or bare spots occur in the coating. The coating so produced is also intimately adherent to the face of the mold and yet it does not cake; it is relatively inert to the cast metal; and it does not crack, flake, blister, or become displaced or roughened by contact of the molten metal therewith. The uniformity of the coating results in a uniformity in its heat insulating effect, thereby reducing chilling of the casting to a uniform extent throughout the surface of the mold. Furthermore, because of the very uniformity of the coating, the casting will duplicate relatively fine and intricate designs on the mold surface with precision.

While in its broader aspects the present invention thus involves the coating of centrifugal molds for casting iron or steel pipes, tubes, etc., as hereinbefore described, a preferred procedure involves preliminarily treating the mold by applying a plurality of coatings as heretofore described and buffing the surface of each coating after the vehicle has been volatilized therefrom, until by such plurality of coatings a relatively thick and

permanent coating has been formed on the mold surface. Thereafter a single coating of the colloidal-graphite-mineral-oil mixture is applied to the mold surface in advance of each casting operation, as in the manner first above described, and experience has demonstrated that by so proceeding the amount of colloidal graphite removed during each casting operation approximates that deposited during the latter coating operation, so that on the one hand the coating does not tend to build up, while on the other hand a permanent coating effected by the aforesaid preliminary treatment remains on the surface of the mold. Thus the life of the mold is materially increased while the use of the plurality of buffed coats results in an improved casting having a surface which is substantially uniform in the physical and chemical characteristics of its surface and which is also possessed of a smooth shiny surface of greatly improved appearance. When the last described procedure is followed, any suitable number of coats may be applied in building up the permanent coating on the mold, and while it is not essential that every coat be subjected to a buffering operation, the preferred procedure involves subjecting each coating to a rubbing or buffering operation so that the permanent coating so formed on the surface of the mold is by reason of its treatment and constitution provided with a highly polished, smooth surface.

It will therefore be perceived that by the present invention an improved method for treating iron or steel molds for the centrifugal casting of iron or steel pipes, tubes, etc., has been provided which realizes each and all of the foregoing objects and which produces a casting of improved character and appearance. Owing to the uniformity with which the coating material is applied to the mold, and the manner in which it is applied, not only are blow holes, blisters and other irregularities avoided on the surface of the casting, but by reason of the character of coating employed, the uniformity of its insulating capacity because of the use of graphite of such particle size and so distributed, the uniformity of the action of the graphite on the molten metal, etc., the casting has uniform physical and chemical characteristics at its surface as well as a smooth polished surface of greatly improved appearance.

While the preferred procedure of the present invention has been described with considerable particularity it is to be expressly understood that the invention is not restricted thereto, as changes may be made in the details of procedure, apparatus used, etc., and certain features may be used without other features, and changes may be made in the temperatures, pressures, degrees of dilution of the colloidal mixture or solution, relative speeds of application of the coating material, etc., to meet the exigencies of particular situations, all as will be apparent to those skilled in the art. Reference is therefore to be had to the appended claims for a definition of the invention.

What is claimed is:

1. The method of preparing metal molds for use in the centrifugal casting of iron or steel pipes, tubes, or the like, which includes maintaining relative movement between the mold and a source of coating material composed of colloidal graphite suspended in a vehicle of volatile oil, distributing over the inner face of said mold a substantially uniform layer of said coating material of sufficient thickness that the suspended

graphite therein will provide a continuous layer of graphite over the inner face of the mold, and effecting deposition of said graphite on and adherence of said graphite to the inner face of the mold by volatilizing said volatile oil.

2. The method of preparing metal molds for use in the centrifugal casting of iron or steel pipes, tubes, or the like, which includes maintaining relative rotary and axial movement between a spraying device and the mold, spraying onto the inner face of said mold a substantially uniform layer of coating material composed of colloidal graphite suspended in a vehicle of volatile oil such that the suspended graphite therein will provide a continuous layer of graphite over the inner face of the mold, and effecting deposition of said graphite on and adherence of said graphite to the inner face of the mold by volatilizing said volatile oil.

3. The method of preparing metal molds for use in the centrifugal casting of iron or steel pipes, tubes, or the like, which includes as a preliminary to each casting operation maintaining relative movement between a hot mold and a source of coating material composed of colloidal graphite suspended in a vehicle of volatile oil, distributing over the inner face of said mold a substantially uniform layer of said coating material such that the suspended graphite therein will provide a continuous layer of graphite over the inner face of the mold, utilizing the heat of the mold to volatilize said volatile oil and effect a substantially uniform deposit of said graphite on and adherence of said graphite to the inner face of the mold, and permitting said coating to dry thoroughly before casting thereon.

4. The method of preparing metal molds for

use in the centrifugal casting of iron or steel pipes, tubes, or the like, which includes as a preliminary to each casting operation rotating the mold while still hot from a preceding casting operation, moving a spraying device axially of the mold, spraying on the inner face of the mold a substantially uniform layer of coating material composed of colloidal graphite suspended in a vehicle of volatile oil such that the suspended graphite therein will provide a continuous coating over the inner face of the mold, and utilizing the heat of said mold to volatilize said volatile oil and effect the deposition of said colloidal graphite on and adherence of said colloidal graphite to the inner face of the mold.

5. The method of preparing metal molds for use in the centrifugal casting of iron or steel pipes, tubes, or the like, which includes the steps of maintaining relative movement between the mold and a source of coating material composed of colloidal graphite suspended in a vehicle of volatile oil, building up a permanent coating of colloidal graphite on the surface of the mold by applying successive coats of said coating material to the inner face of the mold and drying each coat before applying the next succeeding coat thereto, and then applying to the surface of said permanent coating a uniformly distributed coating of colloidal graphite suspended in a vehicle of volatile oil and evaporating the volatile oil to deposit a temporary coating of colloidal graphite on the surface of said permanent coating as a preliminary to each casting operation.

6. The method according to claim 5 wherein at least one or more of the dried coats are buffed in advance of applying a succeeding coat thereto.

CLARENCE DALE BARR.